

# UNITED STATES PATENT OFFICE.

GEORGE E. POTTS, OF SHORT HILLS, NEW JERSEY, ASSIGNOR TO THE POTTS POWDER COMPANY, OF NEW YORK, N. Y., A CORPORATION OF NEW JERSEY.

## ART OF MANUFACTURING NITRO COMPOUNDS.

1,008,615.

Specification of Letters Patent. Patented Nov. 14, 1911.

No Drawing.

Application filed July 13, 1911. Serial No. 638,316.

*To all whom it may concern:*

Be it known that I, GEORGE E. POTTS, recently of Reynolds, Pennsylvania, and now of Short Hills, New Jersey, have invented 5 certain new and useful Improvements in the Art of Manufacturing Nitro Compounds, of which the following is a description.

The invention so far has been most useful in connection with the manufacture of nitro-glycerin, gun cotton, pyroxylin, nitro-cellulose, xylonite and smokeless powder, but it will be readily seen that it is equally applicable to the manufacture of many other nitro compounds (meaning compounds with

15  $\text{NO}_2$ ).

After nitrating cellulose, glycerin, etc., it is frequently very difficult to completely purify the nitro compounds to a satisfactory degree, for example, to make them sufficiently stable to pass what is generally known as the English Government heat test, which requires that the material shall be heated for a period ranging from ten to fifteen minutes to a temperature of 160 degrees 20 Fahrenheit, and that under these conditions a piece of paper moistened with a prescribed solution of potassium iodid and starch shall exhibit a color equal to the prescribed standard color in not less than ten or fifteen minutes, or other prescribed time. I have discovered that these nitro compounds will stand a test for much longer periods of time if they are washed with a solution of ferrous salt, such as ferrous sulfate, or similar 25 ferrous salt, for example, chlorid or nitrate, the thorough washing being accomplished by first washing with water to remove excess

acid so far as conveniently practicable and then with a dilute solution of ferrous-sulfate, for example, one part by weight of ferrous-sulfate dissolved in one hundred times the weight of water, which will be sufficient to wash one hundred pounds of nitro compounds. After running off the excess ferrous-sulfate solution, the nitro compound is again washed with water, and, finally, with a solution of an alkali, for example, one pound of carbonate of soda dissolved in one hundred pounds of water for each hundred pounds of the compound to be washed.

What I claim and desire to secure in this process is the following:

1. Improvement in the art of manufacturing a nitro compound, which consists in washing it with water, then washing it with a solution of ferrous-sulfate, then again washing it with water, and with a solution of an alkali.

2. Improvement in the art of manufacturing a nitro compound, which consists in the step of washing it with a solution of ferrous-sulfate.

3. Improvement in the art of manufacturing a nitro compound which consists in the step of washing it with a solution of a ferrous salt, substantially as set forth.

In testimony whereof I have signed this specification in the presence of two subscribing witnesses.

GEORGE E. POTTS.

Witnesses:

F. E. GRISWOLD,  
GEO. W. BANES.